

(No Model.)

W. WILMINGTON.

METHOD OF CASTING CAR WHEELS.

No. 309,120.

Patented Dec. 9, 1884.



WITNESSES:

*W.W. Hollingsworth*  
*Edw. H. Ryan*

INVENTOR:

*Wm. Wilmington*  
BY *Munn L.*

ATTORNEYS.

# UNITED STATES PATENT OFFICE.

WILLIAM WILMINGTON, OF TOLEDO, OHIO.

## METHOD OF CASTING CAR-WHEELS.

SPECIFICATION forming part of Letters Patent No. 309,120, dated December 9, 1884.

Application filed July 10, 1884. (No model.)

*To all whom it may concern:*

Be it known that I, WILLIAM WILMINGTON, a citizen of the United States, residing at Toledo, in the county of Lucas and State of Ohio, have invented certain new and useful Improvements in Methods of Casting Car-Wheels, of which the following is a description.

This invention relates to an improvement upon a method of casting car-wheels, upon which method Letters Patent No. 289,741 of the United States were granted me December 4, 1883. That method consists in placing finely-powdered ferro-manganese or its equivalent gradually in the stream of molten iron from the pouring-ladle or in the receiving-basin of the mold with the molten iron when the mold of the car-wheel is about three-fourths filled, the ferro-manganese being melted by contact with the molten iron and disseminated in the same in the hub and plate portions of the car-wheel. This method produces very beneficial effects upon the iron forming the hub and plate portions of cast-iron car-wheels, but not to the extent desired upon the iron composing the brackets and flange parts of the wheel, because at the time the ferro-manganese, (or its equivalent,) in combination with the inflowing iron, enters the mold the iron already in the same and filling the depressions in the drag forming the brackets and the back part of the flange had become solidified to such an extent as to prevent the ferro-manganese or its equivalent from diffusing itself in these parts; consequently, the iron forming these portions of the wheel remains in its normal state. The objections to the same may be stated as follows: The flange of the car-wheel projects away from the main body of metal forming the rim of the wheel, and the metal forming the flange being inclosed by the chill and moist sand, the molten iron is suddenly solidified, and the same not having its chill-hardening properties modified by the diffusion of ferro-manganese through it, this causes the flange at times to be almost wholly white or chill-hardened, which lessens greatly the strength of the flange, and is very objectionable.

The common method of forming brackets on

the back part of cast-iron car-wheels imparts greater strength to the wheel at a less cost than any other known method; but brackets are to a certain extent objectionable because of their necessary form, the same being comparatively thin, and, projecting away from the plate of the wheel, are, next to the flange, the parts to cool first, and being connected with the hub-plate and rim of the wheel, and the same being in one piece, causes inherent strain upon the car-wheel, which increases the liability of the same to fracture while in use.

The object of my improvement is to overcome these difficulties; and to this end I modify the chill-hardening properties of molten cast-iron forming a car-wheel in varying degrees by a method of imparting rich ferro-manganese to the molten iron immediately before or at the time the iron is entering the mold of a car-wheel from the basin of the same, thus forming an admixture with the molten iron of rich ferro-manganese, or its equivalent, in varying quantities, whereby the iron composing the brackets and flange of the wheel are modified to an extent without materially affecting the tread of the wheel, and at a later period of filling the mold by placing greater quantities of ferro-manganese, or its equivalent, into the inflowing iron forming the hub and inner plates, which will further modify the chilling properties of the iron forming the same.

In practicing my improvement of casting chilled-tread cast-iron car-wheels, I use the common forms of double or single plated car-wheel molds having various forms of depressions in the drag of the same to impart form to a series of brackets, and also the back part of the flange of the wheel. The mold being in a horizontal position, I take in a pouring-ladle a required quantity of molten chill-hardening cast-iron, or other suitable combination of cast-irons and steel for car-wheels, and commence to fill the mold of a car-wheel in the ordinary manner, with the exception or addition of the following process. At the time, or immediately after commencing to fill the mold, I commence to place gradually into the current of molten iron from the pouring-ladle, or into the receiving-basin of the mold with the molt-

55

65

70

75

80

85

90

95

100

en iron, rich and finely-powdered or granulated ferro-manganese, or its equivalent, allowing the same to be melted and disseminated by the inherent heat in the molten iron in the flowing stream of the same or in the basin. The continuous flow of molten iron will carry with it into the mold the ferro-manganese, and the same being diffused in the iron filling the depressions in the drag forming the brackets and flange will modify the chilling properties of the same. The continuing inflow of molten iron at this time having greater quantities of ferro-manganese, or its equivalent, in mixture, finally fills the mold, whereby the iron forming the hub and inner plates is still further modified in its chilling properties, and thus securing to the car-wheel great strength.

To modify the iron forming these parts of cast-iron car-wheels, I prefer to use by my process very rich ferro-manganese, which may be from seventy-five to ninety per cent., because it takes less to produce the desired results; but I do not confine myself to the use of rich ferro-manganese alone to alloy certain parts of cast-iron car-wheels; but I may use to modify the chilling properties of some qualities of chill-hardening cast-iron small particles of spiegeleisen or small particles of cast-iron having large portions of manganese or uncombined carbon in their composition. I also use to alloy, by my process, suitable combinations of cast-iron and steel for chilled-tread car-wheels, any required combination of the above-named alloying metals in such proportions as the quality of the molten product requires to produce the character of car-wheel desired.

I have found in practice that about three ounces of eighty per cent. ferro-manganese to each one hundred pounds of iron in the wheel produces very beneficial effects in modifying

the iron forming portions of cast-iron car-wheels; but I use greater proportions of the alloying equivalents named, the quantity depending upon the chilling properties of the molten product from which the car-wheel is to be cast by my method, as described above.

The accompanying drawing represents a central cross-section of the mold of car-wheel; A, the basin; B, the inflowing openings; C, depressions in the drag forming the brackets; D, another depression in the drag forming the back part of the flange.

The distinctive features of my invention consist in imparting rich ferro-manganese, or its equivalent, to molten chill-hardening cast-iron at or about the time the same is first entering the mold of a car-wheel whereby the projecting portions of the iron of the wheel in the drag are lessened in their chill-hardening properties, and at a later period of the filling of the mold imparting greater quantities of ferro manganese to the iron flowing into the mold.

What I claim as my invention is—

The method of casting car-wheels, which consists in placing gradually into the stream of molten metal or in the receiving-basin of a car-wheel mold at or about the time of the first entering of molten metal product into the mold rich and finely-powdered or granulated ferro-manganese, or its equivalent, whereby the same is melted and disseminated by the inherent heat in the stream of flowing iron, or in the molten iron in the receiving-basin, and at a later period increasing the proportion of ferro-manganese, substantially as and for the purpose described.

WILLIAM WILMINGTON.

Witnesses:

ALEXANDER WEBER,  
LINCOLN HAYS.